

H. FRASCH, DEC'D.  
 E. FRASCH & F. F. WHITON, EXECUTRICES.  
 PROCESS OF AND APPARATUS FOR ROLLING IRON RODS.  
 APPLICATION FILED JUNE 11, 1897.  
**1,118,275.** Patented Nov. 24, 1914.  
 2 SHEETS-SHEET 1.



Attest:

Walter W. Robinson

J. H. Schott

Inventor:

Herman Frasch  
 by Chas. J. Hedrick  
 his attorney

H. FRASCH, DEC'D.

E. FRASCH & P. F. WHITON, EXECUTRICES.

PROCESS OF AND APPARATUS FOR ROLLING IRON RODS.

APPLICATION FILED JUNE 11, 1897.

1,118,275.

Patented Nov. 24, 1914.

2 SHEETS—SHEET 2.



Fig. 3.



Fig. 4.



Fig. 5.



Fig. 6.



Attest:

Instrument maker

J. H. Schott

Inventor:

Herman Frasch  
by Chas. J. Hedrick  
his attorney

# UNITED STATES PATENT OFFICE.

HERMAN FRASCH, OF CLEVELAND, OHIO; ELIZABETH FRASCH, OF NEW YORK, N. Y., AND FRIEDA F. WHITON, OF HEMPSTEAD, NEW YORK, EXECUTRICES OF SAID HERMAN FRASCH, DECEASED.

## PROCESS OF AND APPARATUS FOR ROLLING IRON RODS.

1,118,275.

Specification of Letters Patent. Patented Nov. 24, 1914.

Application filed June 11, 1897. Serial No. 640,366.

*To all whom it may concern:*

Be it known that I, HERMAN FRASCH, a citizen of the United States, residing at Cleveland, in the county of Cuyahoga and State of Ohio, have invented certain new and useful Improvements in Processes of and Apparatus for Rolling Iron Rods; and I do hereby declare the following to be a full, clear, and exact description of the invention.

This invention relates more particularly to the prevention of scale in rolling red hot iron or steel, as in making rods from billets; but some of the improvements may admit of other applications; and each of them is intended to be secured for all the uses to which it may be adapted.

In rolling iron rods, the hot billet is run through rolls, for reducing it in diameter and elongating it, so as to form a rod of the desired diameter; and as ordinarily conducted, the rod in process of formation is so exposed to air and water (in a liquid state or as vapor) as to become coated with a scale, which has to be removed by the aid of acid. This scale formation not only increases the work to be done on the rod; but it results in a considerable loss of iron or steel originally in the billet.

In accordance with the present invention the highly heated metal during the rolling operation, is kept dry (ordinarily it comes in contact with the water which is poured over the rolls to cool them); and the metal particles as they are brought to the surface in the successive reductions and consequent elongations or spreadings of the billet or partly formed rod, as well as during the intervals between the reducing operations, are protected by inclosure in a non-oxidizing atmosphere. When the rolling is finished the rod or other metal article is still at too high a temperature to bear exposure, either to air or water, without undergoing surface oxidation; it is, therefore, according to the present invention, cooled in a non-oxidizing medium.

To carry out this process use is made of a continuous rolling mill, that is to say of a rolling mill which is composed of one or more trains of rolls with means for mechanically conducting the rod (or other article) from pass to pass, so that personal handling by workmen is not required. In such a con-

tinuous mill, the passes (or more advantageously the entire grooves including the passes), as well as the spaces from each pass to the next, are inclosed in a chamber which is filled with an atmosphere free from uncombined oxygen and from such oxygen compounds as, like water, are decomposed by red hot iron.

To avoid drenching the rolls with water, these are made hollow and are provided with an interior water circulation or with other means for keeping them cool from the inside.

For cooling the rolled article without surface oxidation an non-oxidizing cooler is provided which may be a bath of non-oxidizing liquid such as oil, or a chamber which is cooled by a circulation of water or by other cooling medium in its walls or in closed pipes therein, or a chamber filled with a cold non-oxidizing atmosphere, or the like.

To keep the air from entering the protecting chamber of the continuous mill while avoiding waste, the non-oxidizing atmosphere thereof is put under a pressure which almost exactly balances, preferably being very slightly over rather than under, the outside atmospheric pressure. This can be effected by connecting with the protecting chamber a reservoir of the non-oxidizing gas, and providing means for supplying the gas to the said chamber as the pressure begins to fall below that of the outside atmosphere.

In carrying out the foregoing improvements any suitable gas or gases may be used to form the atmosphere enveloping the hot iron in process of rolling and cooling, provided of course such gas or gases are sufficiently free from uncombined oxygen and decomposable oxygen compounds to produce an industrial result. There are, however, special advantages in using combustion gases from a coke or other suitable fire, because said gases are not combustible and can be readily and cheaply produced in unlimited quantities.

Combustion gases, when produced simply by passage of air through a coke fire, are apt to contain uncombined oxygen; and while the percentage of this may not be sufficient to prevent an industrial result, it is sufficient to make desirable a more perfect freedom from uncombined oxygen. To effect its

more complete removal, a combustible gas or vapor such as hydrogen or a volatilized hydrocarbon is mingled with the air, as for example by carbureting the latter, on its way to the gas-producer.

As the result of the reaction in the coke, the oxygen of the air is combined, in part directly with the carbon of the incandescent coke or of the hydrocarbon, in part indirectly with carbon by first uniting (it is believed) with the hydrogen of the hydrocarbon to form water which is then decomposed, thereby giving uncombined hydrogen. At any rate, the result of the reaction is a mixture of nitrogen, carbonic oxide and dioxid and uncombined hydrogen, with practically no oxygen or water. The presence of the uncombined hydrogen in this atmosphere tends to counteract the oxidation of the iron of the rod or billet; and with this object it might be introduced into the gases from the producer as well as into the air on its way thereto.

It is evident that a non-oxidizing atmosphere, from combustion gases prepared as described, could be used to protect hot metal not only in reduction by rolling but in other relations. The invention extends to their preparation for and use in forming a protecting atmosphere for hot metal while being rolled and in other relations. The use of a non-oxidizing atmosphere composed mainly of nitrogen with a smaller proportion of carbonic oxide and dioxid (either or both) and uncombined hydrogen, is also included in the invention. Some steam could be passed with the air through the incandescent coke.

The percentage of water vapor in combustion gases would (as said before) be insignificant; but, for further assurance, or where the gases contain moisture as the result of a cleansing operation or otherwise, they may be dried by passage through or over sulfuric acid or calcium chlorid or other dehydrating agent before admission to the chamber surrounding the reducing rolls.

In the accompanying drawings, which form part of this specification, Figure 1 is a diagram in plan view, partly in section, showing anti-scale rod-rolling apparatus in accordance with the invention. Fig. 2 is a diagram of the apparatus for generating the non-oxidizing atmosphere, partly in section on line  $i-i$  of Fig. 1. Fig. 3 is a diagram of the rolling mill in section on line  $i-i$  of Fig. 1, Figs. 4, 5 and 6 are partial views illustrating somewhat different arrangements, also within the invention, and Fig. 7 is a detail view illustrating in longitudinal section a portion of one of the internally cooled rolls.

As shown in Figs. 1 and 3 there are two trains of rolls A and B respectively, with

tubular rod guides A' or B' between adjacent pairs of rolls of the same train and a platform guide A'' between the trains. The rolls as shown are driven at accelerated speed; and the platform A'' also accommodates the overfeed of the rod by allowing it to form a loop of greater or less length on said platform. For driving the rolls bevel gears 2, shafts 3 underlying the rolls, and spur gears 4 are shown, but any suitable gearing may be used. It is also to be observed that what has been thus far described is simply by way of illustrating a continuous rolling mill, that such mill has of itself no essential novelty and that it may (within the limits of the invention) be replaced by other known or suitable forms of continuous mill or by other like apparatus. The rolls A B are hollow and are provided with means for cooling them internally, which means may be of any suitable description, but are shown as being composed of a cold water pipe C with branches C' leading well into the rolls, (see Fig. 7) and a return pipe D with branches D' leading from the ends of the cavities, the branches passing through suitable stuffing boxes E.

Inclosing the trains of rolls A D are walls F forming a chamber sufficiently gas-tight to confine a non-oxidizing atmosphere therein. As shown in Figs. 4 and 5 this chamber is formed by walls F' in conjunction with the walls of guides A' between the rolls A and the housings A\* of said rolls. Of course the housings of the rolls could be used as a part of the walls of the inclosing chamber independently of the walls of the rod guides and conversely the walls of said guides might form part of the walls of a protecting chamber in conjunction with other walls which might be independent of the roll housings.

In Figs. 4 and 5 the gears for the rolls, as also the water-pipes C D and the stuffing boxes E, are outside of the protecting chamber; and this arrangement has advantages irrespective of the use of the roll housings and rod guides (either or both) as part of the chamber walls. In Figs. 4 and 5 also the protecting chamber is contracted between adjacent pairs of rolls; thereby saving space both inside and outside, and allowing readier access to the rod. Such a contraction could be made without utilizing the roll housings or the walls of the rod guides as a portion of the chamber walls.

In all the forms the protecting chamber incloses the grooves, including the passes, of the rolls, as well as the spaces (occupied by the rod guides A' A'' B') from one pass to the next.

As the rod leaves the last roll of the mill, it is still so hot that it would be oxidized by contact with air or water. To cool it

without oxidation, it is received by a holder G (shown as a long pipe) surrounded by a jacket H to which water or other cooling medium is supplied by means of branches H' of the mains C D or from other suitable source; or as shown in Fig. 6, it may (without coming in contact with air) be immersed in a bath H\* of oil. As shown in this figure there is a guide pipe leading from chamber F down below the level of the coil, and there are guide rollers 5 under the oil. The oil bath or the cooling jacket could be placed within the chamber F instead of outside of it.

15 The gas-producing apparatus shown at the top of Fig. 1 and in Fig. 2 is for supplying a non-oxidizing atmosphere to the chamber F. It consists of an air blower or fan K which delivers air to the combustion chamber of an air-gas-producer K' a portion being diverted on its way through the carbureting vessel K'' which contains petroleum naphtha or other suitable hydrocarbon. The combustion gases then pass 20 through a purifying apparatus of any suitable description, such for example as a condenser L and scrubber L' of the kind common in gas works to the gas holder M. From this a pipe 6 conducts it into the 25 chamber F. All the air might be passed through the carburetor K'' (which may be of any suitable construction) but it is preferred to carburet only to a slight extent. By closing the valve 7 in the by-pass around 30 the carburetor, more or less, a greater or less proportion of the air will be forced through the carburetor.

35 The operation is as follows:—The red hot billet is introduced through the end 40 wall of the protecting chamber to the pass between the first pair of reducing rolls A; and thence it goes successively from pass to pass, being guided mechanically by the rod guides A' A'' B'. As the rolls A B 45 are cooled internally, the metal remains dry during its passage through the mill. At each reduction the metal is spread laterally or longitudinally or both, so that new surfaces of metal are thereby exposed to the 50 atmosphere in the chamber F. To prevent the formation of scale at this time as well as in the intervals between reductions, while the rod is traveling through the guides A' A'' B' from each pair of rolls to the 55 next, the enveloping atmosphere is made of a non-oxidizing character.

Such an atmosphere is furnished by the air-gas from the producer K', the air which is supplied by the fan K, after said air has 60 been mingled with hydrocarbon vapor by passing a portion thereof through the carburetor K'', being brought in contact with incandescent carbon in the said producer K'. Thus a non-oxidizing gas mixture is obtained consisting mainly of nitrogen with

smaller proportions of carbonic acid and dioxide and of hydrogen. This mixture after leaving the condenser L and scrubber L' is delivered to the gasometer M, to be taken thence as required to the protecting 70 chamber F.

In order to prevent air from entering this chamber F, the gas therein is subjected to pressure, by suitably loading or counter-balancing the bell of the gas holder M, so 75 that the barometric pressure within the chamber balances or very slightly over-balances that of the atmosphere outside of said chamber.

The rod from the last roll B, is cooled 80 to a non-oxidizing temperature while still kept out of contact with uncombined oxygen and decomposable oxygen compounds, such as water. As shown in Figs. 1 and 3, the cooling would be effected by the water circulating in the jacket H of the pipe G (whose interior is occupied by a non-oxidizing atmosphere). As shown in Fig. 6, it is cooled by direct immersion in a bath of a 85 non-oxidizing liquid, such as oil.

In consequence of an official requirement to divide the application for the present patent, a divisional application has been filed, to wit, on September 28, 1914, No. 863,969, for the herein above disclosed improvements in the manufacture of gases and gaseous atmospheres of non-oxidizing 95 character.

I claim as my invention or discovery:

1. The improvement in hot-rolling iron or 100 steel consisting in subjecting the highly heated iron or steel in a dry state to successive reducing operations, and protecting the freshly exposed iron or steel surfaces by an atmosphere free from uncombined 105 oxygen and from oxygen compounds which are decomposable like water by highly heated iron or steel, the protection by said atmosphere being continued as well during the intervals between reductions as while 110 the iron or steel is undergoing the reducing operations, substantially as described.

2. The improvement in hot-rolling iron or steel, consisting in subjecting the highly heated iron or steel in a dry state to successive reducing operations, protecting the freshly exposed iron or steel surfaces by an atmosphere free from uncombined oxygen and from oxygen compounds which are decomposable like water by highly heated iron 115 or steel, and cooling the reduced metal under the protection of a non-oxidizing medium, the iron or steel being protected by the aforesaid atmosphere as well during the intervals between reductions as while 120 the iron or steel is undergoing the reducing operations, substantially as described.

3. The improvement in hot-rolling iron or steel, consisting in subjecting the highly heated iron or steel in a dry state to succes- 130

sive reducing operations, and protecting the freshly exposed iron or steel surfaces by a non-combustible atmosphere free from uncombined oxygen and from oxygen composed mainly of nitrogen with smaller proportions of carbonic acid and dioxide and uncombined hydrogen, substantially as described.

5 pounds which are decomposable like water by highly heated iron or steel, the protection by said atmosphere being continued as well during the intervals between reductions as while the iron or steel is undergoing the 10 reducing operations, substantially as described.

4. The improvement in protecting hot metal from oxidation, consisting in enveloping the same in a non-oxidizing atmosphere having the composition and properties of the gaseous products from passing air mingled with a combustible hydrogen-containing gas or vapor in contact with incandescent carbon, substantially as described.

15 5. The improvement in protecting hot metal from oxidation, consisting in enveloping the same in a non-oxidizing atmosphere having the composition and properties of the gaseous products from passing air mingled with hydrocarbon vapor in contact with incandescent carbon, substantially as described.

20 6. The improvement in hot rolling iron or steel, consisting in subjecting the highly heated iron or steel in a dry state to successive reducing operations, and by means of a non-oxidizing atmosphere having the composition and properties of the gaseous products from passing air mingled with a combustible hydrogen-containing gas or vapor in contact with incandescent carbon, protecting the metal surfaces as they are freshly exposed by the said reducing operations and during the intervals between reductions, substantially as described.

25 7. The improvement in hot rolling iron or steel, consisting in subjecting the highly heated iron or steel in a dry state to successive reducing operations, and by means of a non-oxidizing atmosphere having the composition and properties of the gaseous products from passing air mingled with hydrocarbon vapor in contact with incandescent carbon, protecting the metal surfaces as they are freshly exposed by the said reducing operations and during the intervals between reductions, substantially as described.

30 8. The improvement in hot rolling iron or steel, consisting in subjecting the same highly heated in a dry state to successive reducing operations, and by means of a non-oxidizing atmosphere composed mainly of nitrogen with smaller proportions of carbonic acid and dioxide and uncombined hydrogen protecting the metal surfaces as they are freshly exposed by the said reducing operations and during the intervals between reductions, substantially as described.

35 9. The improvement in protecting hot

metal from oxidation, consisting in developing the same in a non-oxidizing atmosphere composed mainly of nitrogen with smaller proportions of carbonic acid and dioxide and uncombined hydrogen, substantially as described.

70

10. The improvement in hot-rolling iron or steel, consisting in subjecting the highly heated iron or steel in a dry state to successive reducing operations, and protecting the freshly exposed iron or steel surfaces by an atmosphere of air from which with the aid of carbon free oxygen has been eliminated, substantially as described.

75

11. The improvement in hot rolling iron or steel, consisting in subjecting the highly heated iron or steel in a dry state to successive reducing operations, and protecting the freshly exposed iron or steel surfaces by an atmosphere of air from which free oxygen has been eliminated, the last portions of free oxygen having been eliminated by admixture of a small proportion of combustible gas or vapor and exposure of the mixture to an elevated temperature, substantially as described.

90

12. The improvement in hot-rolling iron or steel consisting in subjecting the highly heated iron or steel in a dry state to successive reducing operations by surfaces cooled artificially by conduction from an inclosed cooling medium, and protecting the freshly exposed iron or steel surfaces by an atmosphere free from uncombined oxygen and from oxygen compounds which are decomposable like water by highly heated iron or steel, the protection by said atmosphere being continued as well during the intervals between reductions as while the iron or steel is undergoing the reducing operations, substantially as described.

105

13. The improvement in hot-rolling iron or steel, consisting in subjecting the highly heated iron or steel in a dry state to successive reducing operations by surfaces cooled artificially by conduction from an inclosed cooling medium, and protecting the freshly exposed iron or steel surfaces by a non-combustible atmosphere free from uncombined oxygen and from oxygen compounds which are decomposable like water by highly heated iron or steel, the protection by said atmosphere being continued as well during the intervals between reductions as while the iron or steel is undergoing the reducing operations, substantially as described.

110

14. The improvement in hot rolling iron or steel, consisting in subjecting the highly heated iron or steel in a dry state to successive reducing operations, protecting the iron or steel in process of reduction by a medium less oxidizing than the ordinary air of rolling mills, and cooling the rolled iron or steel under the protection of such a

115

120

125

medium by means of cooling fluid inclosed within heat conducting walls, substantially as described.

15. The improvement in hot rolling iron or steel, consisting in subjecting the highly heated iron or steel in a dry state to successive reducing operations, and protecting the freshly exposed iron or steel surfaces by a non-combustible atmosphere of air from which free oxygen has been eliminated by the aid of carbon, substantially as described.

16. Apparatus for hot rolling iron or steel, comprising metal rolling means whereby the highly heated iron or steel can be subjected in a dry state to successive reducing operations, gas supplying means whereby aeriform fluid free from uncombined oxygen and from oxygen compounds which are decomposable like water by highly heated iron or steel can be supplied in appropriate volume to form a protecting atmosphere within the apparatus, and gas retaining means whereby such aeriform fluid can be retained in contact with the iron or steel, said means of the several kinds mentioned being combined and arranged for protecting the iron or steel by said atmosphere as well during the intervals between reductions as while the iron or steel is undergoing the reducing operations, substantially as described.

17. Apparatus for hot rolling iron or steel, comprising metal rolling means whereby the highly heated iron or steel can be subjected in a dry state to successive reducing operations, gas supplying means whereby aeriform fluid free from uncombined oxygen and from oxygen compounds which are decomposable like water by highly heated iron or steel can be supplied in appropriate volume to form a protecting atmosphere within the apparatus, gas retaining means whereby such aeriform fluid can be retained in contact with the iron or steel, and metal cooling means whereby the reduced metal can be cooled under protection of a non-oxidizing medium, said means of the several kinds mentioned being combined and arranged for protecting the iron or steel by said atmosphere as well during the intervals between reductions as while the iron or steel is undergoing the reducing operations, and also during the subsequent cooling, substantially as described.

18. Apparatus for hot rolling iron or steel, comprising metal rolling means whereby the highly heated iron or steel can be subjected in a dry state to successive reducing operations, gas supplying means whereby non-combustible aeriform fluid free from uncombined oxygen and from oxygen compounds which are decomposable like water by highly heated iron or steel can be supplied in appropriate volume to form a protecting atmosphere within the apparatus,

and gas retaining means whereby such aeriform fluid can be retained in contact with the iron or steel, said means of the several kinds mentioned being combined and arranged for protecting the iron or steel by said atmosphere as well during the intervals between reductions as while the iron or steel is undergoing the reducing operations, substantially as described.

19. Apparatus for protecting hot metal from oxidation, comprising metal holding means whereby the hot metal can be supported, gas supplying means whereby aeriform fluid having the composition and properties of the gaseous products from passing air mingled with a combustible hydrogen-containing gas or vapor in contact with incandescent carbon can be supplied in appropriate volume to form a protecting atmosphere within the apparatus, and gas retaining means whereby such aeriform fluid can be retained in contact with hot metal, said means of the several kinds mentioned being combined and arranged for enveloping the hot metal in said protecting atmosphere, substantially as described.

20. Apparatus for protecting hot metal from oxidation, comprising metal holding means whereby the hot metal can be supported, gas supplying means whereby aeriform fluid having the composition and properties of the gaseous products from passing air mingled with hydrocarbon vapor in contact with incandescent carbon can be supplied in appropriate volume to form a protecting atmosphere within the apparatus, and gas retaining means whereby such aeriform fluid can be retained in contact with hot metal, said means of the several kinds mentioned being combined and arranged for enveloping the hot metal in said protecting atmosphere, substantially as described.

21. Apparatus for hot rolling iron or steel, comprising metal rolling means whereby the highly heated iron or steel can be subjected in a dry state to successive reducing operations, gas supplying means whereby aeriform fluid having the composition and properties of the gaseous products from passing air mingled with a combustible hydrogen-containing gas or vapor in contact with incandescent carbon can be supplied in appropriate volume to form a protecting atmosphere within the apparatus, and gas retaining means whereby such aeriform fluid can be retained in contact with the iron or steel, said means of the several kinds mentioned being combined and arranged for protecting the iron or steel by said atmosphere as well during the intervals between reductions as while the iron or steel is undergoing the reducing operations, substantially as described.

22. Apparatus for hot rolling iron or steel,

- comprising metal rolling means whereby the highly heated iron or steel can be subjected in a dry state to successive reducing operations, gas supplying means whereby aeriform fluid having the composition and properties of the gaseous products from passing air mingled with hydrocarbon vapor in contact with incandescent carbon can be supplied in appropriate volume to form a protecting atmosphere within the apparatus, and gas retaining means whereby such aeriform fluid can be retained in contact with the iron or steel, said means of the several kinds mentioned being combined and arranged for protecting the iron or steel by said atmosphere as well during the intervals between reductions as while the iron or steel is undergoing the reducing operations, substantially as described.
23. Apparatus for hot rolling iron or steel, comprising metal rolling means whereby the highly heated iron or steel can be subjected in a dry state to successive reducing operations, gas supplying means whereby aeriform fluid consisting mainly of nitrogen with smaller proportions of carbonic oxide and dioxid and uncombined hydrogen can be supplied in appropriate volume to form a protecting atmosphere within the apparatus and gas retaining means whereby such aeriform fluid can be retained in contact with the iron or steel, said means of the several kinds mentioned being combined and arranged for protecting the iron or steel by said atmosphere as well during the intervals between reductions as while the iron or steel is undergoing the reducing operations, substantially as described.
24. Apparatus for protecting hot metal from oxidation, comprising metal holding means whereby the hot metal can be supported, gas supplying means whereby aeriform fluid consisting mainly of nitrogen with smaller proportions of carbonic oxide and dioxid and uncombined hydrogen can be supplied in appropriate volume to form a protecting atmosphere within the apparatus, and gas retaining means whereby such aeriform fluid can be retained in contact with hot metal, said means of the several kinds mentioned being combined and arranged for enveloping the hot metal in said protecting atmosphere, substantially as described.
25. Apparatus for hot rolling iron or steel, comprising metal rolling means whereby the highly heated iron or steel can be subjected in a dry state to successive reducing operations, gas supplying means whereby air from which with the aid of carbon free oxygen has been eliminated can be supplied in appropriate volume to form a protecting atmosphere within the apparatus, and gas retaining means whereby such aeriform fluid can be retained in contact with the iron

or steel, said means of the several kinds mentioned being combined and arranged for protecting the freshly exposed iron or steel surfaces by said atmosphere, substantially as described.

26. Apparatus for hot rolling iron or steel, comprising metal rolling means whereby the highly heated iron or steel can be subjected in a dry state to successive reducing operations, gas supplying means whereby air from which free oxygen has been eliminated can be supplied in appropriate volume to form a protecting atmosphere within the apparatus, the last portions of free oxygen being eliminated by admixture of a small proportion of combustible gas or vapor and exposure of the mixture to an elevated temperature, and gas retaining means whereby such aeriform fluid can be retained in contact with the iron or steel, said means of the several kinds mentioned being combined and arranged for protecting the freshly exposed iron or steel surfaces by said atmosphere, substantially as described.

27. Apparatus for hot rolling iron or steel, comprising metal rolling means which include reducing rolls with surfaces cooled artificially by conduction from an inclosed cooling medium, gas supplying means whereby aeriform fluid free from uncombined oxygen and from oxygen compounds which are decomposable like water by highly heated iron or steel can be supplied in appropriate volume to form a protecting atmosphere within the apparatus, and gas retaining means whereby such aeriform fluid can be retained in contact with the iron or steel, said means of the several kinds mentioned being combined and arranged for protecting the iron or steel by said atmosphere as well during the intervals between reductions as while the iron or steel is undergoing the reducing operations, substantially as described.

28. Apparatus for hot rolling iron or steel, comprising metal rolling means which include reducing rolls with surfaces cooled artificially by conduction from an inclosed cooling medium, gas supplying means whereby non-combustible aeriform fluid free from uncombined oxygen and from oxygen compounds which are decomposable like water by highly heated iron or steel can be supplied in appropriate volume to form a protecting atmosphere within the apparatus, and gas retaining means whereby such aeriform fluid can be retained in contact with the iron or steel, said means of the several kinds mentioned being combined and arranged for protecting the iron or steel by said atmosphere as well during the intervals between reductions as while the iron or steel is undergoing the reducing operations, substantially as described.

29. Apparatus for hot rolling iron or steel, comprising metal rolling means whereby the highly heated iron or steel can be subjected in a dry state to successive reducing operations, gas supplying means whereby aeriform fluid less oxidizing than the ordinary air of rolling mills can be supplied in appropriate volume to form a protecting atmosphere within the apparatus, cooling means whereby the rolled iron or steel can be cooled under protection of a non-oxidizing medium, and gas retaining means whereby such aeriform fluid can be retained in contact with the iron or steel, said means of the several kinds mentioned being combined and arranged for protecting by said atmosphere the iron or steel in process of reduction and also the rolled iron or steel during the subsequent cooling, substantially as described.

30. Apparatus for hot rolling iron or steel, comprising metal rolling means where-

by the highly heated iron or steel can be subjected in a dry state to successive reducing operations, gas supplying means whereby non-combustible aeriform fluid consisting of air from which free oxygen has been eliminated by the aid of carbon can be supplied in appropriate volume to form a protecting atmosphere within the apparatus, and gas retaining means whereby such aeriform fluid can be retained in contact with the iron or steel, said means of the several kinds mentioned being combined and arranged for protecting the freshly exposed iron or steel surfaces by said atmosphere, substantially as described.

In testimony whereof I affix my signature, in presence of two witnesses.

HERMAN FRASCH.

Witnesses:

T. W. LOTHMAN,  
J. C. UPDEGROVE.

Corrections in Letters Patent No. 1,118,275.

It is hereby certified that in Letters Patent No. 1,118,275, granted November 24, 1914, upon the application of Herman Frasch, of Cleveland, Ohio, for an improvement in "Processes of and Apparatus for Rolling Iron Rods," errors appear in the printed specification requiring correction as follows: Page 1, line 69, for the article "an" read *a*; page 3, line 10, for the word "coil" read *oil*; page 4, lines 65-66, for the word "developing" read *enveloping*; and that the said Letters Patent should be read with these corrections therein that the same may conform to the record of the case in the Patent Office.

Signed and sealed this 15th day of December, A. D., 1914.

[SEAL.]

J. T. NEWTON,

*Acting Commissioner of Patents.*